

Aug. 4, 1959

S. T. ZEGLER

2,898,252

METHOD OF HEAT-TREATING URANIUM-SILICON ALLOYS

Filed July 3, 1951



INVENTOR.

Sylvester T. Zegler

BY

Roland A. Anderson  
Attorney

1

2,898,252

## METHOD OF HEAT-TREATING URANIUM-SILICON ALLOYS

Sylvester T. Zegler, Chicago, Ill., assignor to the United States of America as represented by the United States Atomic Energy Commission

Application July 3, 1951, Serial No. 234,919

10

8 Claims. (Cl. 148—13)

This invention deals with alloys, in particular with uranium alloys, and with a process of manufacturing said alloys.

The main object of this invention is a uranium-base material which is of great dimensional stability and which in particular does not elongate or otherwise permanently expand after heat-treatment so that it is useful as structural material when it is exposed to periodic temperature changes.

The uranium-base material of this invention is also suitable for use in a neutronic reactor of the type described in the copending application of Fermi et al., Serial No. 568,904, filed December 19, 1944, and granted as U.S. Patent No. 2,708,656 on May 17, 1955.

It has been found that by incorporating a small quantity of silicon into the uranium metal and subjecting the alloy obtained thereby to rolling in the alpha phase, which is below about 660° C., heating the rolled metal at beta phase-temperatures, which are between about 660° and 770° C., and then quenching the alloy, for example, by immersion in water, a material is obtained that is of great dimensional stability and in particular does not expand when alternately heated and cooled.

A silicon content of from 0.01 to 0.1% by weight was found to have this favorable effect; however, from 0.05 to 0.07% by weight of silicon is the preferred range, and 0.07% has given the optimal results. The binary uranium alloy containing 0.07% by weight of silicon showed even a contraction when subjected to the above-mentioned heat-treatment provided that the beta-treatment was carried out long enough. For many uses of uranium a contraction under the influence of alternate heating and cooling is less objectionable than expansion.

In order to show the effect of silicon and also of variation in heating times in the beta phase, a number of comparative experiments were carried out with a uranium-silicon alloy having 0.07% by weight of silicon on the one hand and with pure uranium on the other hand. In all instances the uranium and uranium alloy, respectively, were rolled at 600° C. into rods of a diameter of 0.45" and a length of 2". After the rolling step, the rods were immersed in a lead bath of 600° C. for five minutes in order to preheat the metal and subsequently to obtain the beta phase temperature in a shorter period of time. Thereafter, the rods were immersed into another lead bath of 700° C. and left there for periods of time varying within a range of between two and one hundred twenty seconds. The samples were then quenched in water (room temperature) and finally annealed for two hours at 575° C. in an atmosphere of argon gas. The annealing step is not obligatory in order to obtain the properties desired.

The rod samples thus treated after centerless grinding to provide smooth surfaces were examined for dimensional stability. For this purpose they were cycled repeatedly between a minimum temperature of 100° C.

2

to a maximum temperature of 550° C., the heating period to the higher temperature being carried out within five minutes, while twenty minutes were allowed each time for cooling to 100° C. The tests were carried out using a total of 509 cycles with intermediate examinations. The results of these experiments are compiled in the following table.

| Compound   | $\beta$ -Treatment Time at 700° C.,<br>secs. | Percent Change in Original Length after— |            |            |
|------------|----------------------------------------------|------------------------------------------|------------|------------|
|            |                                              | 100 cycles                               | 300 cycles | 509 cycles |
| 100% U     | 2                                            | 1.47                                     | 2.47       | 3.5        |
| 100% U     | 5                                            | 1.56                                     | 2.65       | 4.3        |
| 100% U     | 10                                           | 1.72                                     | 2.97       | 4.9        |
| 100% U     | 20                                           | 1.44                                     | 4.03       | 5.7        |
| 100% U     | 30                                           | 0.18                                     | 0.39       | 1.03       |
| 100% U     | 60                                           | 0.16                                     | 0.57       | 0.83       |
| 100% U     | 120                                          | 0.22                                     | 0.67       | 1.07       |
| 0.07% Si/U | 2                                            | 4.97                                     | 9.30       | 15.0       |
| 0.07% Si/U | 5                                            | 4.42                                     | 10.35      | 15.9       |
| 0.07% Si/U | 10                                           | 0.34                                     | 0.80       | 1.1        |
| 0.07% Si/U | 20                                           | -0.24                                    | -0.87      | -1.50      |
| 0.07% Si/U | 30                                           | -0.18                                    | -1.04      | -1.81      |
| 0.07% Si/U | 60                                           | -0.15                                    | -1.34      | -2.32      |
| 0.07% Si/U | 120                                          | -0.15                                    | -0.68      | -1.12      |

It will be seen from this table that after a treatment of twenty seconds in the beta phase a contraction (negative elongation) rather than expansion took place when the alloy was subjected to the cycling treatment used.

The results of the lower half of this table were plotted in a diagram in which the times of beta-treatment are shown on the abscissa and the elongation (in percent) of the heat-treated uranium-silicon rods on the ordinate. The curves obtained, as shown in the attached drawing, all cut the zero line, which represents no elongation or contraction during thermal cycling at the same point, namely, at that corresponding to a beta-treatment time of fifteen seconds. This means, in other words, that if the rods are subjected to a temperature of 700° C. for fifteen seconds, an absolutely dimensionally stable material is obtained.

It will be understood that this invention is not to be limited to the details given herein but that it may be modified within the scope of the appended claims.

What is claimed is:

1. A process for manufacturing uranium-base material of a high degree of dimensional stability, and in particular free from thermal expansion, comprising incorporating into the uranium silicon in an amount such as to obtain a content of from 0.01 to 0.1% by weight, rolling the alloy obtained at a temperature of below 660° C., beta-heating said alloy to a temperature of between 660° and 770° C., and quenching the alloy.
2. The process of claim 1 wherein the silicon content ranges from 0.05 to 0.07% by weight.
3. The process of claim 1 wherein the silicon content is 0.07% by weight.
4. The process of claim 1 wherein the material is rolled at about 600° C.
5. The process of claim 1 wherein beta-heating is carried out at about 700° C. for at least ten seconds.
6. The process of claim 5 wherein beta-heating is carried out for fifteen seconds.
7. The process of claim 1 wherein the quenching is carried out with water of room temperature.
8. The process of claim 1 wherein the quenched alloy is annealed for approximately two hours at 575° C. in an atmosphere of argon.

References Cited in the file of this patent

UNITED STATES PATENTS

70 1,601,931 Van Arkel Oct. 5, 1926

(Other references on following page)

## UNITED STATES PATENTS

1,719,975 Gero July 9, 1929  
2,574,626 Daane et al. Nov. 13, 1951  
2,574,627 Daane et al. Nov. 13, 1951

## OTHER REFERENCES

Tucker, Jr.: "The Crystal Structures of Metallic Uranium," AEC Document No. AECD-2716, dated July 21, 1949, declass. September 23, 1949, pp. 1-14.  
Chipman: "Metallurgy in the Development of Atomic Power," AEC Document No. MDDC-539, dated October

1946, declass. November 25, 1946, pp. 12, 13, 14 especially relied upon; entire publication contains 20 pages.

5 Wilson et al.: X-Ray Studies of Alpha, Beta and Gamma Uranium," AEC Document No. AECD-2046, declass. June 9, 1948, page 3 especially relied upon; entire document contains 8 pages.

6 Zachariasen: "The Crystal Structure of Uranium Silicides and of CeSi<sub>2</sub>, NpSi<sub>2</sub> and PuSi<sub>2</sub>"; AEC Document No. AECD-2092, dated January 6, 1948, declass. June 28, 1948, pp. 1-11.